

July 28, 1959

C. VILLORESI

2,896,692

METHOD OF MAKING CUSHIONING PAPER

Filed Nov. 22, 1954

4 Sheets-Sheet 1

*Fig. 1.*



*Fig. 2.*



*Fig. 3.*



*Fig. 4.*



*Fig. 5.*



*Fig. 6.*



Inventor:  
Camillo Villoresi,  
By Stevens, Davis, Miller & Kauff-  
mann, Attorneys

July 28, 1959

C. VILLORESI

2,896,692

METHOD OF MAKING CUSHIONING PAPER

Filed Nov. 22, 1954

4 Sheets-Sheet 2



Fig. 7



Fig. 9



Fig. 10



Fig. 11



INVENTOR

Camillo Villoresi

BY Stevens, Davis, Miller + Maher

ATTORNEYS

July 28, 1959

C. VILLORESI

2,896,692

## METHOD OF MAKING CUSHIONING PAPER

Filed Nov. 22, 1954

4 Sheets-Sheet 3



Fig. 18.



Fig. 16.



## *Inventor:*

Camillo Villaresi,  
by Stevens, Davis, Kellogg & Son  
Attorneys.

July 28, 1959

C. VILLORESI

2,896,692

## METHOD OF MAKING CUSHIONING PAPER

Filed Nov. 22, 1954

4 Sheets-Sheet 4



INVENTOR

*Camillo Villoresi*

BY Stevens Davis Miller & Neuber

ATTORNEYS

# United States Patent Office

2,896,692

Patented July 28, 1959

1

2,896,692

## METHOD OF MAKING CUSHIONING PAPER

Camillo Villoresi, Milan, Italy, assignor to Societa per Azioni Fabbriche Fiammiferi ed Affini, Milan, Italy, a corporation of Italy

Application November 22, 1954, Serial No. 470,469

7 Claims. (Cl. 154—33.05)

This invention relates to formed papers for wrapping, packing, and display and other decorative purposes, and their method of manufacture, and pertains more particularly to the type of papers which are corrugated, pleated, fluted, or otherwise preformed to impart rigidity and cushioning properties. The present application is a continuation-in-part of my copending application Serial Number 244,049, filed August 28, 1951, now abandoned.

One of the common types of paper used for protective packaging is that ordinarily known as "single-faced corrugated paper" and consists of a corrugated sheet attached to a flat backing sheet. A plain corrugated sheet in which the corrugations run in straight lines in the usual manner has very little rigidity or resistance to crushing. The corrugations can be easily flattened, and the paper can be readily pulled out straight in the direction transverse to the corrugations. For this reason a flat backer is ordinarily glued or pasted to one side or to both sides of a corrugated sheet in order to retain the shape and position of the corrugations. The laminated sheet which is thus produced is inelastic, and relatively inflexible, in all directions, and its use is thus limited to packaging flat articles, forming boxes, and other applications for which a stiff, flat sheet is suitable.

One of the principal objects of this invention is to provide a cushioning paper which, in one of its forms, has a rigidity and resistance to crushing comparable, or superior to that of the usual single-faced or double-faced corrugated paper of the same weight, and, in another form, has a high degree of rigidity in one direction while being readily flexible, extendible, and elastic in another direction so that it can be wrapped around circular or irregularly shaped articles and will conform closely to the shape of such articles.

Another principal object of this invention is to provide a method of producing a cushioning paper which has the properties just described, and which permanently retains these properties without a backer or facing sheet. Other objects are to provide a method of permanently impressing undulations into paper, and of subsequently gathering the paper into folds running along the general direction of the undulations and compressing the folds to any desired degree of tightness according to the properties which are required for a particular purpose.

The paper here described, in its basic form, has its undulations disposed in zigzag lines, instead of the straight lines conventionally employed in standard corrugated paper. The zigzag rows of undulations are preferably of uniform width and their mean course is disposed along parallel lines running in a direction which will be here referred to as the "transverse" direction of the paper. The direction in the general plane of the paper perpendicular to the transverse direction will be referred to as the "longitudinal" direction. In the basic form the paper is highly resistant to crushing in a direction perpendicular to its general plane, is substantially inelastic in both longitudinal and transverse directions, and is highly resistant to buckling or bending in the transverse direction. It is moderately flexible, that is, it can be bent on a fairly large radius, in the longitudinal direction, but its rigidity, without a backing sheet, is nevertheless comparable to that of conventional corrugated paper formed from the same type of stock, with a backing sheet at-

2

tached. In this form the paper is useful for protecting flat articles, for lining boxes, and for any of the other purposes for which conventional corrugated paper is used.

For many uses and applications, instead of having the paper completely rigid, that is, substantially inelastic in both longitudinal and transverse directions, it is desirable to have the paper flexible and elastic in the longitudinal direction, while still resistant to crushing in a direction perpendicular to its general plane and stiffer in the transverse direction. Such form of the paper is obtained by initially impressing the paper with the zigzag lines or corrugations as in the basic form, and then pressing or gathering the paper in a longitudinal direction so as to bring the corrugations closer together in such direction. The pressing of the corrugations results in an increase in the height or vertical dimensions thereof, considered perpendicular to the horizontal plane of the paper and a decrease in the horizontal dimension or width, thus longitudinally of the paper, of the corrugations. The inclined faces of the zigzag undulations or corrugations rotate around axes centrally intersecting the faces and paralleling transverse lines running alternately along the peaks and valleys of the corrugations, intermediate the points of the zigzags. The faces rotate about such axes, while moving bodily relative towards each other about the transverse lines. The zigzag undulations then appear somewhat flattened, as they lie on sloping walls to either side of the transverse lines which serve as fold lines but the angular formation has not been changed in actuality, the right angle of the zigzag has not changed. In this form, the paper is more resistant to crushing, and stiffer in the transverse direction than in the basic form, but is flexible and elastic in the longitudinal direction. It is far superior in crush resistance and transverse rigidity than, for example, ordinary pleated paper, and has the further characteristic that it tends to spring back into shape after it is stretched in the longitudinal direction, that is, about the transverse fold lines. In this form, the paper is an excellent cushioning wrapper for round or irregularly shaped articles, as it conforms readily to the contours of such articles.

The process is carried out in one or more stages or steps, there being five stages here described. The first stage, which is essential for making the basic form of the paper, comprises the impressing of zigzag undulations or corrugations in parallel rows across the paper with a predetermined spacing arrangement. As used herein, the words "undulations" and "corrugations" are synonymous, and refer to and describe the formations termed "bas-reliefs" in my aforesaid co-pending application, the term "bas-reliefs" being also synonymous with the words "undulations" and "corrugations."

The impression is primarily a heat molding process rather than a stamping or embossing process and is carried out by the use of an apparatus which includes a pair of heated cooperating rolls, each of which has peripheral rows of chevron-like teeth. The rolls are rotatably disposed with their teeth in meshing engagement and paper is loosely fed into the bite of the rolls with very little tension being imposed on the paper and only enough to maintain the paper straight. The paper has a natural small moisture content and passes between the meshing teeth of the rolls and around a substantial part of the circumference of one of the rolls. A curved plate or shield is disposed about the part of the circumference of the one roll and the paper travels between the roll and the plate or shield which is slightly spaced from the roll. It is believed that a permanent set is made in the paper because of the heated meshing teeth and the proximity of the paper to one of rolls following the meshing teeth engagement of the paper and that the moisture in the

paper forms steam under the initial contact of the paper with the meshing teeth, and the steam produces a barrier or spacer between the roll and the paper and between the shield and the paper. The shield prevents the paper from oxidizing while imparting a permanent resilient set to the paper after the initial impression had been made by the meshing teeth. The steam rising from the paper on the initial engagement of the paper with the meshing teeth is believed to be channeled by the circumference of the roll and the shield to form an insulating barrier which protects the paper from the roll and shield. The shield, because of its close proximity to the paper and structural arrangement thereof with the roll, excludes from contact with the sheet of paper all air except for the small amount of air which may enter in the space between the sheet and the shield. This small residual amount of air is insufficient to support combustion, and, furthermore, as stated above, at least part of this residual air is driven out by steam emitted from the paper. The substantial exclusion of air and the insulating effect of the steam barrier, resultant from moisture in the paper, are believed to be factors in preventing scorching or burning of the paper. The shield forms a curing chamber with the upper roll and the steam in such chamber pushes out the air so as to prevent oxidation. The paper has the impressions molded therein in passing through the bite of the rolls. The heated rolls in pressing the paper upset the fibers and alternate and reposition or realign them and the "set" or mold is cured and made permanent by the passage of the paper through the curing chamber. In such chamber, the steam rising from the paper at the bite of the rolls expands and pushes out and excludes air.

The paper, thus, has the rows of corrugations permanently set therein and the rows are preferably so spaced that straight lines can be passed transversely of the paper and centrally along the mean course of the peaks and troughs of the corrugations. Such lines serve in the other stages of the process as fold lines about which the paper is gathered.

In the second stage of the process the paper is longitudinally gathered with the paper folding about the fold lines and the corrugations being brought closer together in a longitudinal direction of the paper. In the third stage the folds or pleats are further compressed, each fold being moved closer toward the other but without destroying the zigzag corrugations and, in the fourth stage, the folds are compressed still further in a longitudinal direction to form a very-tight succession of undulated folds. A fifth stage may follow the fourth stage and consists of stretching the paper in a longitudinal direction to obtain an intermediate degree of tightness. Dependent on the desired final characteristics of the paper, the various stages will be employed and all or any one of the stages subsequent to the first stage may be omitted.

In the drawings illustrating the best known form of the invention:

Fig. 1 is a schematic view of the apparatus used to carry out the first stage of the process;

Fig. 2 is an enlarged detail elevational view of a portion of the surface of one of the rolls and showing a typical tooth formation;

Fig. 3 is an enlarged cross-section of a portion of the impressing rolls in the region of their meshing bite with the tooth portions of a pair of meshing discs shown in elevation;

Fig. 4 is a plan view of the basic form of the paper produced by the first stage of the method;

Fig. 5 is a cross-sectional view taken on line 5—5 of Fig. 4;

Fig. 6 is a cross-section taken along line 6—6 of Fig. 5;

Fig. 7 is a schematic view of suitable apparatus for carrying out the second and third stages of the process;

Fig. 8 is a plan view, somewhat enlarged, of the paper as it emerges from the second stage;

Fig. 9 is an edge view of the paper shown in Fig. 8, drawn to the same scale as Fig. 7;

Fig. 10 is a schematic view of the apparatus for carrying out the first, second, third and fourth stages;

Fig. 11 is a plan view, somewhat enlarged, of the very tightly folded product produced by the first four stages of the method;

Fig. 12 is an edge view of the paper shown in Fig. 11, drawn to the same scale as Fig. 7;

Fig. 13 is a schematic plan view of a small piece of the product shown in Fig. 11;

Fig. 14 is a schematic view of apparatus for carrying out the fifth stage as well as the first four stages of the process;

Fig. 15 is an enlarged longitudinal section of a modification of the paper produced by the first stage.

Fig. 16 is an enlarged plan view of the modification 20 of Fig. 15;

Fig. 17 is a side view of a bottle wrapped in the elastic form of the paper;

Fig. 18 is a top plan view of the paper product in its basic form and is similar to, but on a larger scale than 25 Fig. 16;

Fig. 19 is a longitudinal sectional view taken on line 19—19 of Fig. 18;

Fig. 20 is a longitudinal sectional view similar to Fig. 19 but showing the paper in a transitional stage between 30 the first stage and the second stage or repressing step;

Fig. 21 is a longitudinal sectional view of the paper of Fig. 18 after the performance of the repressing step or the emergence of the paper from the second stage of the method, the section being taken on a line at the same 35 point of the paper as Fig. 19;

Fig. 22 is a longitudinal sectional view of the paper after the second stage and is taken on a line spaced transversely of the line on which Fig. 21 is taken; and

Fig. 23 is a longitudinal sectional view of the paper 40 after its emergence from the third stage.

The apparatus for performing the basic operation includes suitably internally heated, cooperating impressing rolls 15 and 16 and a shield 17 which is disposed around a substantial part of the upper roll 15.

45 The rolls are positively and synchronously driven in the direction of the arrows by any conventional means (not shown). These rolls are provided with meshing teeth having chevron-like shape, as shown in Fig. 2. The rolls are preferably made up of sets of disks arranged in pairs as, for example, disks 18 and 19. The pairs may be slightly spaced to provide grooves 20 which accommodate stripper fingers 21 and 22 at the bottom and top of the upper roll. The paper sheet 23 is fed in the direction of the arrow 24 and passes between the meshing teeth of the rolls and around the upper roll until it emerges from the upper edge of the shield plate at the top of the upper roll.

50 The paper is preferably fed at very light tension, the tension being merely sufficient to keep the sheet straight; the paper is thus gathered rather freely into the teeth which mesh fairly loosely, as shown in Fig. 3. Preferably one of the rolls, for example, the lower roll 16, is made adjustable up and down, so that the meshing clearance 55 can be readily varied according to the thickness of the paper to be formed. The mesh is set very loose at the start of operations and a few trial sheets are run through. The rolls are gradually brought into closer mesh until a trial sheet appears uniformly impressed to the desired depth. If the mesh is too close, small cuts will appear in the paper indicating that the rolls should be moved further apart. The temperature of the rolls may vary from about 100° C. to 480° C., according to the nature 60 of the paper fed to the machine.

The plate 17 is set very close to the upper roll, with just enough clearance over the thickness of the paper so that the paper lying over the points of the teeth will slide by the plate freely, but close enough so that the paper cannot spring away from the roll. On emerging from the upper roll the paper has the general appearance illustrated in Figs. 4 and 5, and Figs. 15, 16, 18 and 19. The difference between the shape of the zigzag patterns of Figs. 4 and 18 is the result of a difference in the shape of the ends of the teeth. The teeth forming the corrugations of Fig. 4 are rounded somewhat at their ends while the teeth forming the corrugations of Fig. 18 have flatter ends.

The zigzag rows of corrugations 25 impressed in the sheet have a high degree of permanency and will retain their shape without a backing sheet. In the heavier kraft papers, for example, the corrugations will spring back into shape after the paper is twisted or pressed a number of times. Even fairly thin papers, such as glassine, retain the impression with a considerable degree of permanency. The "rigid" form of the product illustrated in Fig. 4 and Figs. 16 and 18 can, therefore, be used in place of the usual types of laminated corrugated paper for packaging flat articles, lining boxes, and many other applications. The elimination of the backing sheet and the pasting operation, which is required for making ordinary corrugated paper, makes this product very inexpensive.

Various kinds of paper, ranging, for example, from heavy kraft or strawboard to tissue and glassine, can be successfully treated by this process. Other materials, such as the various synthetic resin sheet materials, and paper backed metal foils which are widely used as wrappers can also be processed in this manner as can fabrics and other materials. Any such papers or other material may be and preferably are fed to the machine in double ply or multiple ply.

The rigidity and permanency of the corrugations impressed by the process just described appears to be due in part to the zigzag arrangement of the corrugations and in part to a heat molding effect which occurs. The reasons for the latter effect are not entirely understood. It is believed, however, that the relatively long contact of the paper with the upper impressing roll, as compared to the momentary contact which occurs in conventional corrugating and embossing operations, combined with the relatively high temperature of the roll imparts a "permanent set" to the corrugations. It has been found that the paper, in this process, will withstand temperatures which would ordinarily cause charring and discoloration. This is due to the cooperation between the roll 15 and the shield, the latter performing three functions in association with the roll. First of all, the shield serves to guide the paper and is disposed close enough to the roll so that the paper cannot spring away from the roll. The shield retains the paper in contact with the heated roll throughout the length of the shield. Secondly, the shield forms a channel with the roll and it excludes air from the channel and from the paper moving in the channel. Thirdly, since the paper has a natural small moisture content, steam is produced upon the pressure contact of the meshing teeth at the bite of the rolls with the paper and this steam moves on both sides of the paper through the channel and is maintained by the periphery of the roll 15 and the shield in contact with the paper to form an insulating barrier between the paper and the roll and between the paper and the shield. It is believed that the air exclusion factor and steam insulating barrier factor are the reasons why the possibility of oxidation is avoided.

The roll temperature required for performing the impressing operation depends on the type of stock to be processed and the speed at which it is run through. In general, the temperature should be as high as the stock will withstand without damage or discoloration. The optimum temperature for any particular material can be

readily determined by running a few test samples at the desired operating speed, and varying the temperature until a satisfactory product is obtained. By way of example, a temperature of 325° C. is suitable for kraft, chip, or straw paper run at 180 feet a minute through rolls of about one foot diameter. This temperature is substantially higher than that heretofore used in corrugating or otherwise forming papers of this general type.

As shown in Figs. 4 and 6, the zigzag corrugations are so arranged that the paper remains substantially straight along lines 26, which are the median lines of the peaks and along lines 26a which are the median lines of the valleys. This arrangement is not essential in the rigid form of the product. If the paper is to be used in the rigid form, the zigzags of successive peak lines may overlap or may be spaced further apart than in the example shown. The position of the median lines, however, is important in carrying out further steps in the process to produce the elastic form of paper, for the median lines serve as fold lines along which the paper is pleated.

The position of the median lines referred to above is shown more clearly in the form of the rigid paper, illustrated in Figs. 15 and 16 and in Figs. 18 to 23. This paper is produced in the manner already described, the only difference being that the roll teeth are cut with flatter ends, so that the resulting corrugations are trapezoidal in cross-section, and the peak and trough regions appear as substantially flat zigzag strips. In Fig. 16, the numerals 40 refer to the peak or top strips, the numerals 41 to the trough or bottom strips, and the numerals 42 and 43 to the sloping side walls connecting the peaks and troughs of the corrugations. It will be noted that lines 26 pass through the adjacent points of the zigzag lines 44 and 45 which define the edges of the peak strips 40. These points will be referred to as the inner vertices of the peak zigzags. Lines 26a likewise pass through the inner vertices of the trough strips, that is, the adjacent points of zigzag lines 46 and 47 which define the edges of the trough strips. The paper

can be creased or folded readily only along the lines 26 and 26a as the shape of the corrugations presents considerable resistance to folding elsewhere. This is important for the performance of further steps in the process which involve reversely folding, or pleating, the paper by gathering it in the longitudinal direction, as the paper will tend to "break" evenly at such natural fold lines and fall into uniform, even pleats. The paper need not lie absolutely straight along lines 26 and 26a but merely straight enough so that the resistance to folding is small

along the median lines 26 and 26a of the peaks and troughs as compared to other regions of the paper. In the form shown in Figs. 4, 5 and 6, for example, in which the corrugations are of more rounded contour, a cross-section along one of the median lines, may appear

slightly wavy, and consequently the fold lines of the pleats, as in Fig. 8 are slightly wavy. It is also apparent that the flat peak and trough strips in the example of Fig. 16 might be slightly wider, in which case the median lines would not pass through the inner vertices of the peak and trough zigzags. The paper would then not be

constrained to fold along exact lines, and it is to be expected that the pleats resulting from further steps of the process would not be exactly even and uniform in depth. As long as the transverse folds are confined to fairly narrow regions, however, to produce the desired degree of uniformity in the pleats, the product would be usable for processing in the manner about to be described.

It is, therefore, understood that any reference herein to the lines 26 and 26a as lying substantially straight, or as running substantially through the inner vertices of the trough and peak zigzags, includes tolerable departures from the exact arrangement illustrated in Figs. 16 and 18 et seq.

In Figs. 18 and 19, the paper is shown in its basic form, as shown in Figs. 15 and 16. The flat top or peak

strips 40 extend transversely across the paper in longitudinally spaced rows and are spaced by the sloping side walls 42 and 43 from the flat bottom or trough strips 41. The lines 26 and 26a pass through the top and bottom strips and form straight fold lines about which the top and bottom strips fold or roll as the side walls rotate and move bodily toward each other. To describe this movement, attention is directed to Figs. 18 through 21, wherein Figs. 20 and 21 are taken on the same line as Fig. 19 and show the movement of the strips and the side walls. The lines 26 centrally intersect the top strips and divide them into rows of staggered isosceles triangles which have their bases lying on the line 26. Thus, the triangles 40A bounded by the angular sections of the side walls 42 have their bases lying on the lines 26 with the triangles 40B bounded by the angular sections of the side walls 43 having their bases on the lines 26. The triangles 40B are in one row in end to end continuing relation at the lines 26 and the triangles 40A in the other row are in end to end continuing relation at the lines 26. The sides of the triangles 40A are bounded by the sloping angular sections of the side walls 42 and the sides of the triangles 40B are bounded by the sloping angular sections of the side walls 43. The bottom strips are similarly divided into contiguous rows of triangles by the median lines 26a. The lines 26 and 26a are thus predetermined fold or hinge lines about which the contiguous rows of triangles rotate. For example, the row of triangles 40A moves down about the line 26 while the row of triangles 40A also moves down about the line 26, until in a final stage, the rows of triangles 40A are substantially vertically disposed alongside the vertically disposed rows of triangles 40B.

This movement is accomplished by a gathering apparatus which gathers the paper longitudinally so that the paper folds about the lines 26 and 26a. The apparatus is shown in Fig. 7 and will be hereinafter described. With the apparatus of Fig. 7, the paper moves about the lines 26 and 26a into pleats or folds.

As shown in Fig. 20, which is a transition stage between stage one (Fig. 19) and stage two (Fig. 21), the gathering action causes the paper to start to break on the lines 26 and 26a. The triangular section 40A moves down about the line 26 with the side wall 42B rotating about itself and moving inwardly. The side wall 43C moves inwardly toward the side wall 42B and rotates about itself. The bottom section 41D moves upwardly about the line 26a.

The lines 26 and 26a form natural breaking lines or predetermined fold lines because the lines have the bases of the triangles lying therein and the lines do not intersect the apexes of the angular side wall sections that bound the triangles. Thus, at such points, along the lines 26 and 26a there is less resistance to folding than at any other points transverse of the paper.

In Fig. 21, the paper is shown as it appears after the completion of the second stage and it will be noted that the lines 26 and 26a form actual break lines. The triangles 40A and 40B have moved down about the line 26 and lie alongside each other on opposite sides of the line 26 but still retain their same angular shape. The side walls have moved closer relative to each other and have moved the triangles of the top strip into parallel association with the corresponding triangles of the bottom strip which also retain their same angular shape.

In Fig. 23, which is a showing of the paper after the completion of the third stage, which is a tighter gathering or repressing stage, the triangles of the top strips and of the bottom strips have been very nearly turned from horizontal to vertical positions, that is perpendicular to the positions they occupied in Fig. 18 and the side walls have begun to nest together.

Fig. 22 is a view similar to Fig. 21 but taken at a point along the paper slightly spaced transversely of Fig. 21. In Fig. 22, the apexes of the triangles 40B are shown

while the points between the triangles 40A are shown so that the walls 42B are fully illustrated.

In this respect, Figs. 20-23 are taken through the apexes of the triangles 40A and, therefore, through the points of touching connection of the triangles 40B so that the side walls 43C are completely shown in association with the corresponding triangles 41D of the bottom strips.

It will be noted that the lines 26 are moved closer together longitudinally of the paper as are the lines 26a, while the lines 26 and 26a are moved further apart vertically of the paper. The lines 26 are closer together in Fig. 23 than in Figs. 21 and 22 and the lines 26a are also closer together in Fig. 23 than in Figs. 21 and 22. The closer the lines are together is dependent on the degree of repressing or gathering and the closer they are together, longitudinally of the paper, the further they are apart vertically.

The second step of the process is shown in Fig. 7. The paper, as it emerges from between roll 15 and plate 17, passes over a plate 30, which may be an extension of the stripper fingers 22, and under a roll 27 which is disposed above the inner end of the plate. The roll 27 is mounted on a swinging arm 28 which is spring pressed toward the paper, for example by means of a spring 29. It is understood that any convenient means for mounting the roll 27, and applying yielding pressure to the roll, may be employed. The roll 27 is preferably knurled on its peripheral surface so that it produces a drag on the paper in the longitudinal direction and tends to brake the motion of the paper. As the result of this braking action, the paper tends to fold into pleats along the natural fold lines 26 and 26a. It then appears as shown in Figs. 8 and 9 and Figs. 21 and 22. It will be noted that the zigzags of the peaks appear somewhat flattened in the longitudinal direction, due to the fact that the corrugations now lie on the sloping sides of the pleats. The lines 26 and 26a are brought closer together longitudinally of the paper while being moved further apart perpendicularly of the paper so that the overall thickness of the paper has been increased. The paper now appears as a series of pleats 33, with the initial zigzag corrugations forming ripples 34 from side to side along the sides of each pleat. This is the basic "elastic" form of the product. In this form it is highly flexible in the longitudinal direction, that is about a transverse axis, but is very stiff in the transverse direction and considerably more resistant to crushing than the form of Fig. 4. In its elastic form the paper is highly suitable for wrapping round, or irregularly shaped articles. For example, Fig. 17 shows a bottle wrapped in this form of paper. The paper will stretch readily around the bulge of the bottle, and yet the stretched part retains its cushioning properties. The paper is truly elastic, rather than merely extensible, in the longitudinal direction, because the rippled structure imparted by the original zigzag corrugations tends to draw the pleats back into shape when the paper is released after stretching. This elasticity may also be due in part to the impression of the folds while the paper is still at high temperature.

Further stages of the process are directed to produce varying degrees of tightness of the folds in the elastic form of the product. The third step is performed by means of a plate 31 which is mounted alongside of roll 27 and above plate 30. Plate 31 is preferably mounted with up and down adjustment and is moved up out of contact with the paper, when only the first two stages of the process are being performed. To perform the third stage, plate 31 is brought down so that it is spaced from plate 30 by a distance to barely clear the paper as it emerges from roll 27. Even though there is slight clearance, the movement of the paper will cause it to drag slightly on one or the other of the plates. This slight drag will compress the pleats in the longitudinal direction and increase the depth of the pleats sufficiently so

that both plates will frictionally engage the paper. The resulting product is shown in Fig. 23.

To perform the fourth stage of the process, a second spring pressed drag roll 35 is mounted alongside plate 31. This roll tends to crowd the pleats between plates 31 and 30 so that they are further compressed in the longitudinal direction. The resulting product is a very tight, almost solid mass of pleats which still exhibit the ripples due to the initial zigzag formation of the corrugations. The ripples of successive pleats are nested one within the other, as illustrated in the schematic view of two pleats shown in Fig. 13, and this interlocking effect imparts high rigidity to the product. This product is extremely rigid in the transverse direction and very difficult to crush, because of its solid structure, but it will still bend readily about transverse lines 25 and 26a, as shown by the reverse bends of the sample illustrated in Fig. 12. In Fig. 12 the paper is shown somewhat stretched for sake of clarity. Fig. 13 more nearly illustrates the structure in its relaxed condition.

The fifth stage is a stretching stage which is used to produce an intermediate degree of tightness. As shown in Fig. 14, the paper is fed to a pair of stretching rolls 36 which are positively driven in the direction of the arrows at a speed faster than the travel of the paper. The speed of the rolls may be varied to stretch the paper to any desired degree. A product of a tightness intermediate that produced by any of the preceding stages may thus be obtained. The fifth stage may be employed immediately after the second, third or fourth stages, as desired.

In carrying out the process through any number of its stages, two or more sheets of paper may be fed to the impression rolls at once, to produce a laminated sheet. The laminations may, if desired, be secured together in the usual manner by paste or other adhesives. One of the interesting properties of this form of paper, however, is the fact that the laminations tend to interlock, due to the peculiar zigzag structure of the initial corrugations. This tendency is most pronounced in the tighter elastic forms of the product. The laminations will thus cling together without adhesive, and the pasting operation can be eliminated for most purposes. This not only results in a saving but also makes it possible to use colored papers of all kinds without danger of smearing and spotting. A wide variety of attractive two-color papers may be produced by laminating in this manner. These products are suitable for window displays, lamp shades, fancy wrappers, and a number of other uses.

I claim:

1. The method of forming a cushioning sheet material which comprises feeding a moisture-containing sheet of deformable material between a pair of intermeshing impression members heated to a temperature between 100° C. and 480° C., to form initially impressed parallel zig-zag rows of corrugations in the sheet, moving the impressed sheet in continuing contact with one of said members through a confining channel immediately adjacent said one member, while maintaining the temperature of said one member within said range, and simultaneously causing the formation of steam within said channel by evaporating the moisture of the heated sheet therein, so that the steam confined in said channel tends to force air from the channel and from the depressions of said sheet, thereby to prevent scorching of the sheet and cause the initial impressions of said sheet to receive a more permanent set.

2. The method described in claim 1, wherein the sheet material is paper, the impression members are rotating rolls, and the paper sheet is relieved of tension while being fed to said impression rolls.

3. The method of forming a cushioning sheet material which comprises feeding a moisture-containing sheet of deformable material between a pair of rotating intermeshing impression rolls heated to a temperature between

100° C. and 480° C., to form initially impressed parallel zigzag rows of corrugations in the sheet, moving the impressed sheet in continuing contact with one of said rolls through a shielded confining channel immediately adjacent said one roll, while maintaining the temperature of said one roll within said range, and simultaneously causing the formation of steam within said channel by evaporating the moisture of the heated sheet therein, so that the steam confined in said channel tends to force air from the channel and from the depressions of said sheet, thereby to prevent scorching of the sheet and cause the initial impressions of said sheet to receive a more permanent set.

4. The method described in claim 3, wherein the sheet is then moved forwardly beyond said channel and away from said one roll, and the sheet is caused to be creased transversely on lines disposed along the troughs and peaks of the corrugations in the mean direction of the rows, by retarding such forward movement of the sheet.

20 sheet.

5. The method described in claim 4, wherein said forward movement of the sheet is retarded by yieldingly pressing a drag roll against one surface of the sheet after it is moved away from said one roll.

25 6. The method described in claim 5, wherein the creased sheet is gathered and pleated by next moving the sheet between a pair of plates frictionally engaging opposite sides of the sheet, to retard its forward movement, and finally further retarding said movement by yieldingly  
30 pressing the creased and pleated sheet between a second drag roll and one of said plates, to compress its pleats, so that portions of adjacent rows of corrugations are nested together.

7. The method of forming a cushioning sheet material which comprises feeding a moisture-containing sheet of deformable material between a pair of rotating intermeshing impression rolls heated to a temperature between 100° C. and 480° C., to form initially impressed parallel zigzag rows of corrugations in the sheet, moving

40 parallel zigzag rows of corrugations in the sheet, moving the impressed sheet in continuing contact with one of said rolls through a shielded confining channel immediately adjacent said one roll, while maintaining the temperature of said one roll within said range, and simultaneously causing the formation of steam within said channel by evaporating the moisture of the heated

45 channel by evaporating the moisture of the heated sheet therein, so that the steam confined in said channel tends to force air from the channel and from the depressions of said sheet, thereby to prevent scorching of the sheet and cause the initial impressions of said sheet to receive

50 a more permanent set, moving the impressed sheet forwardly beyond said channel and away from said one roll, and causing the sheet to be creased transversely on lines disposed along the troughs and peaks of the corrugations in the mean direction of the rows, by yieldingly pressing 55 a drag roll against one surface of the sheet after it is moved away from said one roll, to retard said forward movement, and then stretching the creased sheet in a direction at right angles to the creases thereof, to expand the sheet longitudinally.

**References Cited in the file of this patent**

UNITED STATES PATENTS

|              |           |                |
|--------------|-----------|----------------|
| 657,100      | Ferres    | Sept. 4, 1900  |
| 810,891      | Thiebaut  | Jan. 23, 1906  |
| 85 1,150,805 | Beran     | Aug. 17, 1915  |
| 1,240,231    | Lumley    | Sept. 18, 1917 |
| 1,975,548    | Ives      | Oct. 2, 1934   |
| 2,042,243    | Watson    | May 26, 1936   |
| 70 2,141,235 | Angeletti | Dec. 27, 1938  |
| 2,160,677    | Romanoff  | May 30, 1939   |
| 2,499,267    | Conner    | Feb. 28, 1950  |
| 2,514,801    | Sapp      | July 11, 1950  |

## FOREIGN PATENTS

Italy ----- Feb. 12, 1948